

Patented Apr. 13, 1926.

1,580,189

# UNITED STATES PATENT OFFICE.

STEWART J. CARROLL, OF ROCHESTER, NEW YORK, ASSIGNOR TO EASTMAN KODAK COMPANY, OF ROCHESTER, NEW YORK, A CORPORATION OF NEW YORK.

## CELLULOSE NITRATE COMPOSITION.

No Drawing.

Application filed July 9, 1924. Serial No. 724,935.

To all whom it may concern:

Be it known that I, STEWART J. CARROLL, a citizen of the United States of America, residing at Rochester, in the county of Monroe and State of New York, have invented 5 certain new and useful Improvements in Cellulose-Nitrate Compositions, of which the following is a full, clear, and exact specification.

10 This invention relates to nitrocellulose compositions containing chlorinated derivatives of the cyclic hydrocarbons  $C_{2n}H_{n+3}$  and their homologues.

One object of the invention is to provide 15 a composition of this kind in which the presence of camphor is not required. Another object of the invention is to provide a relatively inexpensive composition in which the flowing and setting properties are 20 enhanced by the use of one or more of the monohydroxy aliphatic alcohols containing more than 3 and less than 6 carbon atoms. Other objects will hereinafter appear.

In U. S. Patent No. 1,342,602, Seel, June 25 8, 1920, cellulose nitrate composition, there is disclosed a flowable film-forming composition in which cellulose nitrate is combined with a chlorinated derivative of certain cyclic hydrocarbons, such as naphthalene, the combination being effected with the aid of both camphor and a monohydroxy aliphatic alcohol, such as butyl alcohol or fusel oil. I have found that the composition may be simplified and rendered less

35 expensive by omitting the camphor entirely and substituting an increased amount of the monohydroxy aliphatic alcohol, the latter preferably being in a proportion greater than at least 20% of the weight of the cellulose nitrate. Moreover this simplification is effected without substituting any high-boiling esters in place of the camphor. Representative high-boiling esters which are used as camphor substitutes are included 40 in the section on "Camphor substitutes" beginning in page 2535 of part 4, Vol. I of "Technology of Cellulose Esters" by E. C. Worden, published in New York, N. Y., by D. Van Nostrand Company in 1921. While

50 I shall hereinafter give specific examples of my invention, it will be understood that these are for purposes of illustration and that the invention is not restricted to these details, except as indicated in the appended 55 claims.

A flowable film-forming composition suitable for the manufacture of films for photographic purposes comprises 100 parts of nitrocellulose, from 20 to 50 (say 40) parts of butyl alcohol or fusel oil, 10 to 50 (say 60 20) parts of commercial monochlornaphthalene dissolved in 300 to 450 parts of a volatile common solvent, such as methyl alcohol or acetone, or a mixture of these in any proportion (say equal parts by weight of 65 each). The proportion of fusel oil or butyl alcohol is, of course, below that which will cause a precipitation of the other ingredients, the range of percentage just given being particularly useful. The butyl alcohol 70 may be any one of the isomers comprised under that name or a mixture thereof. Normal butyl alcohol is preferred. The fusel oil may comprise chiefly one or more 75 of the isomeric amyl alcohols. Of course, a small amount of lower alcohols, such as propyl alcohol or isopropyl alcohol, can be present, provided the bulk of fusel oil or butyl alcohol comprises the ingredients 80 stated above. The monochlornaphthalene 85 may be of the commercial type, the bulk of it boiling between 250° C. and 275° C. (say chiefly around 265° C.). Where it is desired to have a more freely flowable composition, as in lacquers and varnishes, the amount of acetone or methyl alcohol may be increased until the proper degree is reached.

In place of monochlornaphthalene I may 90 wholly or partially substitute a more highly chlorinated body, such as the commercial translucent waxy tetrachlornaphthalene. This contains other chlornaphthalenes, but its chief boiling range is between 310° C. and 340° C. When used alone, instead of displacing only a small part of the monochlornaphthalene, the maximum amount 95 which is recommended is less than the maximum proportion of monochlornaphthalene named hereinabove. When employed as the sole chlorinated body in the mixture, it is preferable to keep it at about 10% of the weight of the cellulose nitrate.

100 These solutions are sufficiently viscous to flow properly during sheet or film manufacture, the volatile ingredients passing off at the right rate to permit the rapid setting of the films without impairing or pitting the product. The resulting films containing the unvolatilized ingredients are flexible, smooth, 105 110

transparent and uniform sufficiently for use as photographic film. The relatively larger proportion of higher alcohols increases the flexibility.

5 Having thus described my invention, what I claim as new and desire to secure by Letters Patent is:

1. A composition of matter consisting of cellulose nitrate, a chlor-nucleo substitution product of the hydrocarbons  $C_{2n}H_{n+3}$  and their homologues, an alcoholic ingredient weighing more than 20% of the weight of the cellulose nitrate, said alcoholic ingredient comprising chiefly a monohydroxy aliphatic alcohol containing more than 3 and less than 6 carbon atoms and sufficient volatile liquid, which is a common solvent of the three hereinabove named ingredients, to render the mixture flowable.
- 10 2. A simplified composition of matter, substantially free from camphor and high-boiling ester substitutes therefor, comprising cellulose nitrate, a chlor-nucleo substitution product of the hydrocarbons  $C_{2n}H_{n+3}$  and their homologues and an alcoholic ingredient weighing from 20 to 50% of the weight of the cellulose nitrate, said alcoholic ingredient comprising chiefly a monohydroxy aliphatic alcohol containing more than 3 and less than 6 carbon atoms.
- 15 3. A simplified flowable film-forming composition of matter, substantially free from camphor and high-boiling ester substitutes therefor, comprising cellulose nitrate, a chlor-nucleo substitution product of the hydrocarbons  $C_{2n}H_{n+3}$  and their homologues and a monohydroxy aliphatic alcohol containing more than 3 and less than 6 carbon atoms.
- 20 4. A simplified flowable film-forming composition, substantially free from camphor and high-boiling ester substitutes therefor comprising cellulose nitrate, monochlornaphthalene and butyl alcohol.
- 25 5. A composition of matter consisting of 100 parts by weight of cellulose nitrate, from 20 to 50 parts of butyl alcohol, from 10 to 50 parts monochlornaphthalene and 300 to 450 parts of methyl alcohol.
- 30 6. As an article of manufacture, a deposited or flowed film, substantially free from camphor and high-boiling ester substitutes therefor, comprising cellulose nitrate, a chlor-nucleo substitution product of the hydrocarbons  $C_{2n}H_{n+3}$  and their homologues, and a monohydroxy aliphatic alcohol containing more than 3 and less than 6 carbon atoms.
- 35 7. As an article of manufacture, a flexible, transparent film, substantially free from camphor, consisting of cellulose nitrate, monochlornaphthalene, and a monohydroxy aliphatic alcohol containing more than 3 and less than 6 carbon atoms.

alcoholic ingredient weighing from 20 to 50% of the weight of the cellulose nitrate, said alcoholic ingredient comprising chiefly a monohydroxy aliphatic alcohol containing more than 3 and less than 6 carbon atoms, and a volatile liquid which dissolves the hereinabove recited ingredients.

40 4. A simplified flowable film-forming composition, substantially free from camphor and high-boiling ester substitutes therefor comprising cellulose nitrate, monochlornaphthalene and butyl alcohol.

45 5. A composition of matter consisting of 100 parts by weight of cellulose nitrate, from 20 to 50 parts of butyl alcohol, from 10 to 50 parts monochlornaphthalene and 300 to 450 parts of methyl alcohol.

50 6. As an article of manufacture, a deposited or flowed film, substantially free from camphor and high-boiling ester substitutes therefor, comprising cellulose nitrate, a chlor-nucleo substitution product of the hydrocarbons  $C_{2n}H_{n+3}$  and their homologues, and a monohydroxy aliphatic alcohol containing more than 3 and less than 6 carbon atoms.

55 7. As an article of manufacture, a flexible, transparent film, substantially free from camphor, consisting of cellulose nitrate, monochlornaphthalene, and a monohydroxy aliphatic alcohol containing more than 3 and less than 6 carbon atoms.

Signed at Rochester, New York this 26th day of June 1924.

STEWART J. CARROLL.